

**TEXTILE TREATMENT WITH NOVEL AQUEOUS DISPERSION TO ACHIEVE WATER-REPELLENT FINISHES**

Nathaniel J. Glade, Somerville, N.J., assignor to American Cyanamid Company, New York, N.Y., a corporation of Maine

No Drawing. Filed May 22, 1956, Ser. No. 586,357

10 Claims. (Cl. 260—21)

The present invention relates to aqueous dispersions of water-repellent agents, their application to textile materials and the resulting water-repellent textile materials.

An object of the invention is to provide improved compositions for imparting water-repellent effects.

Another object of the invention is to provide an improved durable water-repellent agent for textile materials.

A further object of the invention is to provide an improved method for imparting to textile materials a water-repellent finish which is durable to laundering and dry cleaning.

Still another object of the invention is to provide an improved textile material having a water-repellent finish which is durable to laundering and dry cleaning.

Other objects and advantages of the invention will be apparent to those skilled in the art, especially upon consideration of the detailed disclosure hereinbelow.

The present invention concerns an aqueous dispersion of an aminotriazine-aldehyde resinous condensate; a wax-like compound with a melting point above about 100° F. and containing a hydroxylated aliphatic acyl chain of at least 12 carbon atoms; a hydrophilic protective colloid; and one or more emulsifiers of the group consisting of sulfonated and sulfated fatty acids, alcohols and esters with an aliphatic chain of at least 8 carbon atoms, sulfonated lignin, condensation products of polyalkylene polyamines with fatty acids containing 8 carbon atoms, dialkyl alkylol alkylamides quaternary ammonium salts and water-dispersible reaction products of an aliphatic amine containing at least 12 carbon atoms with epichlorohydrin. In addition, it relates to the treatment of textile materials with these novel dispersions and the product of such treatment. Optionally, the compositions may contain a hydrocarbon or ester wax melting about 100° F. in a quantity ranging up to about 4 times the weight of said hydroxylated wax-like compound, and a minor amount of a fatty alcohol with at least 12 carbon atoms in the aliphatic chain is desirable for many purposes.

The resin employed in the novel compositions may be any aminotriazine-aldehyde condensate or mixture of such compounds which is capable of forming either a true solution in water or a colloidal solution exhibiting the characteristic Tyndall haze. These condensates may be either etherified or alkylated with a suitable alcohol like methanol or simple unetherified condensates of an aldehyde and an aminotriazine. A wide variety of the unalkylated and alkylated aminotriazine-aldehyde condensates and their preparation is disclosed in Widmer et al. Patents Nos. 2,197,357 and 2,191,362; and hence need not be repeated here. The triamino- and diaminotriazines are preferred, especially melamine and the guanamines such as acetoguanamine and propioguanamine. Of these, the methyl ethers of methyol melamines provide the optimum results, and these may contain from 1 to 6 mols of combined formaldehyde and 1 to 6 mols of combined methanol per mol of melamine. The combined methanol content does, of course, not exceed the combined formaldehyde content on a molar basis. For

each 100 parts total of the waxy materials described hereinafter, between about 30 and about 600 parts of the aminotriazine resin may be employed and the preferred amount is between about 60 and about 300 parts. The aminotriazine-aldehyde condensate may be employed either in essentially monomeric form or in the partially polymerized colloidal state in acid solution as described in Patents Nos. 2,345,543 and 2,609,307. Textile finishing resins of the urea-formaldehyde and substituted urea-formaldehyde type may not be substituted for the aminotriazine resins in the novel compositions because the finish imparted thereby to textiles has no permanence or durability whatsoever to dry cleaning and laundering.

Optionally, an additional textile finishing agent derived from urea may be employed along with the aminotriazine resin for the purpose of reducing the yellowing which occurs to some extent due to the retention of chlorine by a melamine resin finish on a textile fabric. This is accomplished without any improvement or decrease in the durability or spray rating of textile fabrics finished according to the present invention. Among the suitable agents for decreasing yellowing are essentially monomeric methylated methyol ureas and their water-soluble lower polymers, and the unalkylated and alkylated formaldehyde condensates of alkylene ureas like dimethylol ethylene urea, dimethylol propylene urea, dimethylol trimethylene urea, and their methyl ethers. These substances and their preparation are well understood and they may contain from 1 to 4 mols of combined formaldehyde per mol of urea or urea derivative as well as a combined methanol content ranging from about 20% up to but not exceeding the formaldehyde content on a molar basis. The water-soluble lower polymers of methylated methyol urea may be easily obtained by refluxing with heating about 2.5 mols of paraformaldehyde per mol of urea in a methanol medium for several hours at an alkaline pH, cooling, adding methanol in stoichiometric excess, adjusting the mixture to a moderately acid pH, refluxing for a short period, then stopping the reaction by cooling and adjusting the pH to a moderately alkaline value. These substances may be employed in quantities ranging up to but not exceeding the weight of aminotriazine resin, and it is generally recommended that at least about 6.6 and preferably about 30 to 100% be used, based on the weight of aminotriazine resin, when chlorine retention is a significant problem. For producing a water-repellent effect on porous materials like cloth, leather, etc., it is seldom desirable to have more than a total of 600 parts of urea derivative and aminotriazine-aldehyde condensate in a dispersion containing 100 parts of waxy material or materials.

The hydrophobic component of the novel oil-in-water dispersions is, of course, in the dispersed phase. This water-insoluble wax-like material contains a compound with a melting point above 100° F. and preferably above 150° F. which has a hydroxylated saturated fatty acyl radical of at least 12 carbon atoms and preferably between 16 and 30 carbon atoms. In these substances, one or more hydroxy groups are attached to one or more carbon atoms in the alkyl chain other than the acyl or carboxylic carbon atoms. Thus this component may be a hydroxylated saturated higher fatty acid or an ester thereof with a monohydric or polyhydric alcohol including glycerol. Among the suitable compounds are hydrogenated castor oil which appears to produce the optimum results, hydrogenated ricinoleic mono- and di-glycerides, 9,10-dihydroxystearic acid, methyl, butyl, cetyl and other alkyl esters of hydrogenated ricinoleic acid, lauryl-9,10-dihydroxy stearate, and mixtures thereof.

A certain percentage of a hydrocarbon or an ester wax melting above about 100° F. may be blended with the hydroxylated waxy material with excellent results. In

this hydrocarbon category are included various grades of paraffin, ozokerite, scale wax, micro-crystalline waxes, and so forth. A few examples of suitable ester waxes of natural or synthetic origin are carnauba, japan, montan, candelilla, beeswax and other insect waxes. Refined paraffin wax is preferred when the dispersion is intended for the treatment of light colored textiles and grades melting above about 120° F. are recommended for best results. Mineral waxes are cheaper than hydroxylated fatty acyl compounds; hence, a blend of the two reduces the cost of the textile treatment. In addition, it has been found that within proper limits a hydrocarbon wax actually enhances the water-repellent characteristics of the textile finish and somewhat improves its durability to dry cleaning and laundering. Blends of equal parts of the two waxy materials seem to appear to be the optimum. However, the hydrocarbon or ester wax may desirably constitute from about 5 up to about 80% of the weight of the hydrophobic component; beyond that, the dry cleaning durability of the textile finish suffers.

The treating agent also contains a small quantity of a hydrophilic protective colloid which serves to stabilize the suspension or dispersion. Polyvinyl alcohol appears to provide the best results and the lower viscosity grades are especially recommended; however, a variety of other materials can be used including lower viscosity grades of carboxymethyl cellulose, gum ghatti, gum arabic, gelatin, polyacrylamide, polymethylolacrylamide, polymethacrylamide, polymethylolmethacrylamide, and the like. In general, any hydrophilic protective colloid that is free of rewetting tendencies after drying is suitable in the present invention. Based on the total weight of waxy ingredients, the protective colloids are desirably present in quantities ranging from about 0.5 to about 20% or more on a dry basis.

A higher fatty alcohol containing from about 12 up to 30 or more carbon atoms is an optional but often highly desirable component of the mixture, especially where a hydrocarbon wax is present. This alcohol is thought to act as a coupling agent which improves the miscibility of the hydroxylated waxy material and the mineral wax. More importantly, it is a stabilizer which provides long shelf life for the wax dispersion. This obviates any necessity for preparing the wax dispersion at the place it is to be used, a feature which is often important inasmuch as textile finishing plants, etc. are seldom equipped with good emulsification equipment such as homogenizers. Thus it is possible to sell the ingredients for preparing the novel dispersions as two items having a prolonged storage life, namely an aqueous solution of the aminotriazine resin and an aqueous dispersion of the waxy material. In addition, it appears that the fatty alcohol facilitates the preparation of wax dispersions on a large scale and it is well known that large quantities of wax emulsions are often less stable than smaller laboratory batches. Cetyl alcohol is preferred for the purpose but one or more other saturated and unsaturated fatty alcohols may be employed, including lauryl, myristyl, stearyl, palmitoyl, oleyl, cetoleyl alcohols and the like may be substituted, if desired. The recommended quantities are from about 1 to 6 parts for each 100 parts of total waxy components.

Many emulsifiers or dispersing agents are unsuitable for the present compositions by reason of incompatibility, a tendency toward rewetting after drying, etc. However, certain classes of wetting or dispersing agents have been discovered which produce good results. Among these are sulfonated or sulfated higher fatty acids, alcohols and esters containing an aliphatic chain of at least 8 but seldom over about 30 carbon atoms. Sulfated fatty alcohols are preferred for the purpose and this expression is used herein to include the alkaline metal salts of such materials since this is the form in which they are commonly available in the market. The many suitable materials encompass esters which term is used

herein to include the esters of polyhydric alcohols such as ethylene glycol, glycerine, etc. as well as monohydric alcohols. Moreover, the aliphatic chains of these materials may be either saturated or unsaturated prior to the sulfonation or sulfation treatment. Among the many suitable materials are caprylyl, capryl, lauryl, myristyl, cetyl, and stearyl alcohol sulfates, sulfonated ricinoleyl alcohol, etc., and their alkali salts; methyl, butyl and other alkyl esters of the aforementioned alcohols; sulfated caprylic, lauric, palmitic, stearic, oleic, linoleic, and linolenic acids as well as sulfonated ricinoleic acid and the corresponding mono-, di- and triglyceride derivates. For example, good results are also obtainable with sodium glyceryl monolaurate sulfate and sulfonated castor oil. 15 Sodium lignin sulfonate has been used with success. Also, polyalkylene polyamine condensates of higher fatty acids like the products of reacting diethylene triamine, hexamethylene tetramine, tetraethylene pentamine, hexaethylene septamine and the like with from about 10% 20 up to a full stoichiometric proportion of a long chain fatty acid (8 to 30 carbon atoms) such as capric, lauric, and stearic acids, frequently accompanied by a lower aliphatic acid such as formic or propionic acid in minor proportion; dialkyl alkylol alkylamide quaternary ammonium salts as exemplified by palmitamidoethyl diethyl gamma-hydroxypropyl ammonium chloride, and similar compounds containing two lower alkyl groups of about 1 to 4 carbon atoms, a 1 to 4 carbon alkylol radical, a halogen atom and a radical containing a higher alkylamide of about 8 to 30 carbons combined with a 1 to 4 30 carbon alkyl group; and the water-dispersible reaction products of long chain aliphatic amines containing from 8 to about 22 carbon atoms, like dodecylamine and eicosylamine, with epichlorohydrin can be employed for the purpose. Suitable amine-epichlorohydrin reaction products and their preparation are disclosed in detail in Lundberg application Serial No. 393,246, filed November 19, 1953 (Patent No. 2,753,372) and these may be neutralized with acetic or another lower carboxylic acid 40 for greater stability. The amine-epichlorohydrin molar ratios may range from about 1:2 to 2:1 and this particular group of compounds is preferred for use under acid conditions, as for instance, where the resinous component is in the acid colloid form. Based on the total weight of waxy materials, the dispersing agents described may be present in amounts ranging from about 0.5 to 15%, and for most purposes, between about 1 and about 4% is recommended. Too much may cause unwanted rewetting.

50 In preparing the novel dispersions the hydroxylated waxy material may be melted and thoroughly blended with any hydrocarbon wax or fatty alcohol which may be added at a temperature of 235° F. for example. Meanwhile, the protective colloid may be stirred into about 70 parts by weight of water with heating until it is dissolved; then the dispersing agent may be added and the aqueous phase heated to about 180-195° F. Next, about 30 parts of the molten waxy mixture may be combined with the aqueous phase with vigorous agitation followed by passing the crude emulsion through a homogenizer at 3000 55 lbs. per square inch. After this, the suspension of wax-like material is cooled rapidly to a temperature below about 120° F. For maximum storage stability, the suspension should be stored alone; however, the aminotriazine resin may be added immediately if desired, preferably in the form of an aqueous solution of the resin.

60 The novel compositions may be used in a variety of applications in the textile, paper and leather fields. They are especially intended for the water proofing of porous materials by impregnating the materials with the aqueous dispersion followed by drying and curing to convert the aminotriazine-aldehyde condensate to the substantially water-insoluble state. This curing is accomplished at elevated temperatures of preferably about 200 to 325° F. or even higher if smoking due to vaporizing a portion 65

of the waxy matter from the impregnated material during curing is not objectionable. In compositions containing a colloidal or partially polymerized aminotriazine resin, heating is not required to cure the resin but is usually preferred in commercial operations in order to expedite the drying of the impregnated material.

The present compositions are particularly adaptable to the finishing of textile fabrics including woven and non-woven, knitted and felted materials containing cellulose fibers like cotton, linen, viscose and cuprammonium rayons, animal fibers like wool, mohair, etc., cellulose acetate, silk, and the various synthetic fibers such as nylon of both the adipamide and caprolactam types and other linear polyamides, homopolymers and copolymers of acrylonitrile with vinyl acetate, methyl acrylate, the vinyl pyridines, etc., polyethylene glycol terephthalate and casein fibers. The dispersions may be applied to either fibers or fabrics by any suitable means such as padding, spraying, immersion, roll coating, etc. The treatment of most fabrics is well exemplified by passing the fabric through a dispersion containing from about 2 to about 35% solids and preferably about 10 to about 20% solids with the squeeze rolls adjusted to provide a dry pick up between about 1 and about 35% and preferably between about 5 and about 20% based on the weight of dry fabric. The wet impregnated fabric is then dried and cured, usually but not necessarily in a single operation by heating at between about 200 and about 325° F. for a period between about 15 and about 4 minutes. Where necessary or desirable the curing is catalyzed by the presence of a suitable catalyst known in the art such as magnesium chloride, amine hydrochlorides, diammonium phosphate and other acidic or latent acid accelerators.

The function of the various components in the new composition is not fully understood. There is some reason to believe that during curing, a noncarboxylic hydroxyl group on the hydroxylated wax-like substance reacts with a methoxymethyl or methylol radical in the aminotriazine compound with a splitting off of water or methanol in what is essentially a transesterification reaction. While this theory would appear to be confirmed by the outstanding durability of textile finishes imparted with the present invention, this merely is offered as a possible explanation; and the invention is not limited to this theory since it has not been established with certainty.

For a better understanding of the nature and objects of this invention, reference should be had to the following illustrative examples in which all proportions are stated in terms of weight unless otherwise indicated therein. In addition, all testing of fabrics is carried out by standard methods adopted by the American Association of Textile Chemists and Colorists (AATCC) unless otherwise stated.

Following the procedure outlined above, a series of aqueous wax dispersions is prepared from the following constituents.

6  
TABLE I

|                                          | Wax Dispersions |      |      |      |      |      |
|------------------------------------------|-----------------|------|------|------|------|------|
|                                          | A               | B    | C    | D    | E    | F    |
| Slack wax                                |                 |      |      |      |      | 14.0 |
| Refined paraffin wax (133-135° F., M.P.) | 14.10           | 14.0 | 9.3  | 18.7 | 14.0 |      |
| Hydrogenated castor oil                  | 14.10           | 14.0 | 18.7 | 9.3  | 14.0 | 14.0 |
| Polyvinyl alcohol                        | 1.25            | 0.3  | 0.3  | 0.3  | 3.0  | 0.3  |
| Sodium lauryl sulfate                    | 0.50            | 0.5  | 0.5  | 0.5  | 0.5  | 0.5  |
| Cetyl alcohol                            | 0.90            |      |      |      |      |      |
| Water                                    | 69.15           | 71.2 | 71.2 | 71.2 | 68.5 | 71.2 |

These are finely divided suspensions of the waxy materials in water which are stable indefinitely. In the textile finishing operations described hereinbelow, they are employed in more dilute form in combination with a resinous material of the type described herein. Suitable pad baths are desirably prepared by warming the wax dispersions to about 110° F. while diluting with about half of the water to be added, stirring the resin or aqueous resin solution into the other half of the water at about 80° F. followed by mixing the two liquids and stirring in a conventional quantity of a suitable curing catalyst for the resin.

#### Example 1

A pad bath is made up containing 6.25% of solids from wax dispersion A and 6.25% by weight of methylated trimethylol melamine (67% methylated) prepared similarly to Example 2 in British Patent 566,347 along with a magnesium chloride solution equivalent to 0.75% anhydrous  $MgCl_2$ . Rayon challis, 80 x 80 cotton percale and a 5.5 ounce cotton poplin fabrics are successively padded through this solution using 1 dip and 1 nip to give wet pickups of 93%, 76% and 72%, respectively. All of the fabrics are dried at 225° F. and the rayon is cured for three minutes at 300° F. while the cotton fabrics are cured in a similar oven at 350° F. for 1.5 minutes.

Other samples of the same three fabrics are treated in the same manner using a bath containing the same quantity of resin and catalyst but none of wax dispersion A.

The two cotton poplins are subjected to Stoll flex abrasion tests only and it is found that the sample treated with the resin solution alone stands 99 cycles whereas the material treated with both resin and waxy materials has a rating of 204 cycle.

The rayon challis and 80 x 80 cotton fabrics are tested for wrinkle recovery, tensile and tear strength and water-repellent characteristics along with untreated control samples of the same materials and the following test data are obtained. During a similar trial using wax dispersion A and a larger proportion of ureaformaldehyde resin on rayon challis, it is found that the treated fabric has excellent wrinkle resistance but the initial spray rating is 0.

TABLE II

| Fabric         | Finish      | Wrinkle Recovery, degrees | Grab Tensile Strength, lbs. | Elmendorf Tear Strength, lbs., Warp and Fill | AATCC Spray Ratings |                |                       |
|----------------|-------------|---------------------------|-----------------------------|----------------------------------------------|---------------------|----------------|-----------------------|
|                |             |                           |                             |                                              | Initial             | After 3 Washes | After 3 Dry Cleanings |
| Rayon Challis  | Untreated   | 175                       | 109                         | 6.37                                         | 0                   |                |                       |
| Do             | Resin alone | 227                       | 116                         | 3.55                                         | 0                   |                |                       |
| Do             | Resin+wax   | 215                       | 122                         | 9.91                                         | 90                  | 80             | 70                    |
| 80 x 80 Cotton | Untreated   | 141                       | 91                          | 2.53                                         | 0                   |                |                       |
| Do             | Resin alone | 250                       | 66                          | 1.60                                         | 0                   |                |                       |
| Do             | Resin+wax   | 251                       | 57                          | 2.42                                         | 90                  | 90             | 80                    |

All cotton washes specified herein are conducted at 160° F. for one hour using a solution of 0.1% soap and 0.1% sodium carbonate followed by rinsing at 160° F. and all rayon launderings are carried out at 100° F. for 1 hour using a solution of 0.1% soap followed by rinsing at 100° F.

Except where otherwise specified herein, all dry cleaning operations are for a period of one hour using a hydrocarbon cleaning solvent known as Varsol II.

#### Example 2

A treating bath is made up with equal weights of dimethylol melamine and the solids of wax dispersion A plus 8.44% mixed isopropanolamine hydrochlorides based on the weight of the melamine compound. The same cotton poplin is padded through this bath to a 10% by weight dry pick up followed by drying and curing for 6 minutes at 290° F. The initial spray rating of the treated fabric is 90+ and the value after one hour of laundering is 70 but the finish is not durable to dry cleaning.

#### Example 3

The same cotton poplin is treated with a bath containing equal weights of trimethylol beta-cyanopropio-guanamine and the solids of wax dispersion A along with 3.5% based on the weight of the guanamine-formaldehyde compound of an accelerator comprising essentially diammonium hydrogen phosphate. The drying, curing and test procedures of Example 2 are followed and the finished fabric is found to have spray ratings initially of 80+ and of 70 after one hour of washing. This finish also is not durable to dry cleaning.

#### Examples 4-18

Several fabrics are padded through the various treating baths listed in Table III below. The resin employed in varying concentrations in these baths is the same methylated trimethylol melamine as in Example 1 but a number of different waxy dispersions are used in preparing the baths which all contain 3½% by weight based on the resin solids of a catalyst having diammonium hydrogen phosphate as the essential active ingredient. The expression is adjusted for an 85% wet pick up in all cases and all drying and curing is accomplished in a single operation requiring 6 minutes in an oven maintained at 290° F. In Examples 8 to 18, inclusive, ethylene dichloride is employed in lieu of Varsol II as the dry cleaning agent.

#### Example 19

|                                                                                                                                   | Wt. percent |
|-----------------------------------------------------------------------------------------------------------------------------------|-------------|
| Colloidal methylated trimethylol melamine (resin solids)                                                                          | 5.00        |
| Hydrogenated castor oil                                                                                                           | 2.50        |
| Carnauba wax                                                                                                                      | 2.50        |
| Polyvinyl alcohol                                                                                                                 | 0.22        |
| Cetyl alcohol                                                                                                                     | 0.14        |
| Reaction product of 1 mol octadecylamine with 2 mols of epichlorohydrin with 75% of the amino groups neutralized with acetic acid | 0.19        |
| Water                                                                                                                             | 89.45       |

15 The partially polymerized colloidal melamine resin above is introduced as a 10% aqueous solution exhibiting the characteristic blue Tyndall haze of cationic water-dispersible melamine resin particles aged in acetic acid as described in Patent No. 2,609,307. An all wool flannel fabric and an 80 x 80 cotton percale are passed through a pad bath of the composition listed above containing no catalyst with the squeeze rolls adjusted for a wet pick up of 100%. After drying at 225° F. for 15 minutes, it is found that both fabrics exhibit greatly reduced shrinkage upon laundering in comparison with untreated samples of the same material. In addition, both fabrics have excellent spray ratings which are durable to dry cleaning and to repeated washings.

20

#### Example 20

|                                                  | Wt. percent |
|--------------------------------------------------|-------------|
| Methylated pentamethylol melamine—50% methylated | 10.00       |
| Hydrogenated castor oil                          | 2.50        |
| Candelilla wax                                   | 2.50        |
| Polyvinyl alcohol                                | 0.22        |
| Cetyl alcohol                                    | 0.16        |
| Sodium lauryl sulfate                            | 0.09        |
| Water                                            | 84.53       |

Viscose, silk, and 80 x 80 cotton percale fabrics are 45 passed through a pad bath of the above composition to which 1.2% magnesium chloride (anhydrous basis) has been added as a catalyst with the squeeze roll set for 85% expression. The fabrics are dried and cured in an oven for 6 minutes at 320° F. The resulting finish is 50 found to impart a high degree of durable water repellence coupled with good resistance to shrinkage, wrinkling and tearing.

TABLE III

| Example | Bath Content   |              |             | Fabric         | AATCC Spray Ratings |               |         |                    |  |
|---------|----------------|--------------|-------------|----------------|---------------------|---------------|---------|--------------------|--|
|         | Wax Dispersion | Resin Solids | Waxy Solids |                | Initial             | After Washing |         | After Dry Cleaning |  |
|         |                |              |             |                |                     | 1 hour        | 3 hours |                    |  |
| 4.      | B              | 10           | 5           | 80 x 80 Cotton | 100                 | 100           | —       | 80                 |  |
| 5.      | B              | 10           | 10          | do             | 100                 | 90+           | —       | 80                 |  |
| 6.      | C              | 10           | 10          | do             | 100                 | 90+           | 70-     | 70                 |  |
| 7.      | D              | 10           | 10          | do             | 100                 | 90            | —       | 70                 |  |
| 8.      | E              | 10           | 5           | do             | 100                 | 90+           | —       | 70+                |  |
| 9.      | F              | 5            | 10          | do             | 90+                 | 70+           | —       | 70-                |  |
| 10.     | F              | 10           | 5           | do             | 100                 | 90+           | —       | 70                 |  |
| 11.     | F              | 7.5          | 3.75        | do             | 90                  | 80+           | —       | 70                 |  |
| 12.     | F              | 5            | 2.5         | do             | 80                  | 70            | —       | 70                 |  |
| 13.     | E              | 10           | 5           | Cotton Poplin  | 100                 | 80+           | —       | 70                 |  |
| 14.     | F              | 10           | 5           | do             | 100                 | 90            | —       | 70-                |  |
| 15.     | E              | 7.5          | 5           | Spun rayon     | 90+                 | 80+           | 80      | 80                 |  |
| 16.     | E              | 10           | 5           | do             | 90+                 | 100           | 90+     | 80                 |  |
| 17.     | F              | 7.5          | 5           | do             | 90+                 | 90            | 80      | 70                 |  |
| 18.     | F              | 10           | 5           | do             | 100                 | 100           | 90      | 80                 |  |

## Example 21

|                                                                 | Wt. percent |
|-----------------------------------------------------------------|-------------|
| Methylated pentamethylol melamine—50% methylated                | 4.20        |
| Partially polymerized methylated dimethylol urea—80% methylated | 2.10        |
| Hydrogenated castor oil                                         | 3.15        |
| Refined paraffin wax                                            | 3.15        |
| Polyvinyl alcohol                                               | 0.28        |
| Cetyl alcohol                                                   | 0.20        |
| Sulfonated castor oil                                           | 0.11        |
| Water                                                           | 86.81       |

With 3.5% (based on the total weight of resin solids) of a catalyst comprising essentially diammonium hydrogen phosphate added to the bath, 5.5 ounces cotton poplin is impregnated to pick up 10% solids based on the dry fabric weight. After drying and curing at 290° F. for 6 minutes in an oven, the initial spray rating of the cloth is 90+. Samples subjected to one hour of washing are found to have a spray rating of 80 and other samples exposed to one hour of dry cleaning are rated at 70 in the same test.

## Example 22

|                                 |       |
|---------------------------------|-------|
| Methylated trimethylol melamine | 6.00  |
| Dimethylol ethylene urea        | 3.00  |
| Hydrogenated castor oil         | 2.50  |
| Refined paraffin wax            | 2.50  |
| Gum ghatti                      | 0.27  |
| Sodium ligninsulfonate          | 0.16  |
| Water                           | 85.57 |

Fabrics woven from nylon, polyethylene glycol terephthalate, and an acrylonitrile copolymer (85% acrylonitrile, 7.5% vinyl acetate, 7.5% 2-methyl 5-vinyl pyridine) fibers, respectively, are padded through a treating bath containing the constituents listed according to the procedure of Example 21. All three fabrics are found to have excellent spray ratings of a substantially permanent nature, and the finishes do not exhibit detrimental effects upon exposure to chlorine bleaching.

## Example 23

|                                         |       |
|-----------------------------------------|-------|
| Methylated trimethylol melamine         | 6.00  |
| Methylated dimethylol trimethylene urea | 3.00  |
| Hydrogenated castor oil                 | 5.00  |
| Polyacrylamide                          | 0.22  |
| Sodium ligninsulfonate                  | 0.16  |
| Water                                   | 85.62 |

A polyacrylamide with a viscosity of 10,160 centipoises (Brookfield) at 10% concentration in water is employed as the protective colloid in this dispersion. Viscose rayon gabardine and 80 x 80 cotton percale are impregnated in this bath and cured using the procedure and obtaining the same qualities as in Example 21.

## Example 24

|                                      |       |
|--------------------------------------|-------|
| Methylated trimethylol melamine      | 6.00  |
| Monomeric methylated dimethylol urea | 3.00  |
| Hydrogenated castor oil              | 2.50  |
| Montan wax                           | 2.50  |
| Carboxymethyl cellulose              | 0.22  |
| Sodium ligninsulfonate               | 0.16  |
| Water                                | 85.62 |

Example 22 is repeated using the bath listed to produce fabrics exhibiting the same characteristics including a low degree of chlorine retention upon exposure to bleaches.

10  
Example 25

|                                                               |       |
|---------------------------------------------------------------|-------|
| Methylated pentamethylol melamine—50% methylated              | 10.00 |
| Hydrogenated castor oil                                       | 2.50  |
| Beeswax                                                       | 2.50  |
| Polyvinyl alcohol                                             | 0.22  |
| Cetyl alcohol                                                 | 0.16  |
| Stearamidopropyl dimethyl beta-hydroxyethyl ammonium chloride | 0.09  |
| Water                                                         | 84.53 |

An 80 x 80 cotton fabric is impregnated with the above dispersion following the procedure of Example 22. Again a durable finish with high spray rating is obtained along with good wrinkle resistance and shrink resistance.

## Example 26

|                                                                                                                |       |
|----------------------------------------------------------------------------------------------------------------|-------|
| Dimethylol melamine                                                                                            | 10.00 |
| Hydrogenated castor oil                                                                                        | 2.50  |
| Refined paraffin wax                                                                                           | 2.50  |
| Polyvinyl alcohol                                                                                              | 0.23  |
| Reaction product of 2.9 mols of technical stearic acid per mol of tetraethylenepentamine plus 1.5% acetic acid | 0.56  |
| Water                                                                                                          | 84.21 |

Cotton and viscose rayon fabrics are treated with the above dispersion in accordance with the procedure of Example 21. A wash-durable wrinkle-resistant and water-repellent finish is obtained on both fabrics.

## Example 27

|                                 |       |
|---------------------------------|-------|
| Methylated trimethylol melamine | 5.00  |
| 9,10-dihydroxy stearic acid     | 2.50  |
| Refined paraffin wax            | 2.50  |
| Polyvinyl alcohol               | 0.22  |
| Cetyl alcohol                   | 0.16  |
| Sodium lauryl sulfate           | 0.09  |
| Water                           | 89.53 |

A viscose rayon gabardine, and a cotton percale fabric are passed through the above pad bath and processed in the manner set forth in Example 21. The durable finish on both fabrics is highly water repellent and has good resistance to wrinkling and shrinkage.

## Example 28

|                                                                                                      |       |
|------------------------------------------------------------------------------------------------------|-------|
| Methylated trimethylol melamine                                                                      | 5.00  |
| Hydrogenated castor oil                                                                              | 2.50  |
| Refined paraffin wax                                                                                 | 2.50  |
| Polyvinyl alcohol                                                                                    | 0.22  |
| Cetyl alcohol                                                                                        | 0.14  |
| Acetic acid neutralized reaction product of 1 mol of octadecylamine with 1.4 mols of epichlorohydrin | 0.09  |
| Phosphoric acid                                                                                      | 0.02  |
| Water                                                                                                | 89.53 |

Cotton poplin and cellulose acetate fabrics are finished with this bath according to the procedure of Example 21. The resulting finish has a high degree of durable water repellency coupled with good resistance to shrinkage, wrinkling and tearing.

From the above results, it is apparent that many beneficial advantages are secured by the present invention and a number of unexpected results are encountered. A high degree of water repellency is obtained along with an excellent durability of the finish to washing when aminotriazine-aldehyde resins are used in the combination. In addition, good durability of the water-repellent finish to dry cleaning is obtained when an alkylated aminotriazine resin is selected. On the other hand, similar benefits are not obtainable with ureaformaldehyde resins in combination with the same waxy materials for not even initial water repellency is developed by the treatment. Dimethylol ethylene urea as a substitute can produce a good initial spray rating on the fabric but the finish is

## 11

not durable to either washing or dry cleaning. The present compositions also produce good wrinkle resistance and shrink resistance. On rayon an important advantage is gained in the greatly increased tear strength, for example more than 50% over the untreated fabric, along with a substantial though smaller increase in tensile strength.

In comparing the effects of the novel mixtures with those obtained by the same resins alone in the absence of the hydrophobic components, one particularly strange effect is noted in that addition of the waxy component produces no softening effect. The most important benefits realized over the straight resin treatments are the great improvement in tear strengths ranging from about 50% on cotton to almost 300% on rayon in addition to the water-repellent characteristics and a doubling of the resistance to wear as measured by Stoll's flex abrasion test.

The present invention possesses a significant economic advantage over a well known commercial water repellent containing melamine resin according to Patent No. 2,357,273, especially when a hydrocarbon wax like paraffin is present in a sizable amount. Difficulties have frequently been encountered from the formation of a large quantity of a rather dry foam in pad baths of the prior art water repellent whereas only a small volume of wet foam is formed on treating baths of the novel compositions. Although seldom necessary, the use of suitable defoaming agents is also contemplated herein, and it is well known that these materials are more effective on wet foams than those of a drier nature. The finishes imparted to textiles are substantially equal in water repellency and durability to washing to those obtained with the aforesaid commercial product, and the abrasion resistance of the cloth is greatly improved. Also, the new compositions can be catalyzed with magnesium chloride which is currently the best accelerator for aminotriazine resins in solution, while the prior art water repellent was incompatible with that catalyst.

While there are disclosed herein only a limited number of embodiments of the composition, process and product of the invention, it is possible to produce still other embodiments without departing from the inventive concept set forth, and it is desired, therefore, that only such limitations be imposed upon the appended claims as are stated therein or required by the prior art.

I claim:

1. A composition of matter which comprises an aqueous dispersion of (1) between about 30 and about 600 parts of a resinous component selected from the group consisting of water-soluble aminotriazine-aldehyde resin and aqueous colloidal aminotriazine-aldehyde resins and mixtures of said aminotriazine-aldehyde resins with a water-soluble textile finishing agent selected from the group consisting of methylated methylol ureas, methylol alkylene urea and methylated methylol alkylene urea, said mixtures containing between about 6.6 and about 100% of said textile finishing agent based on the weight of aminotriazine-aldehyde resin; (2) 100 parts of an hydrophobic component selected from the group consisting of a wax-like compound melting above 100° F. containing an hydroxylated aliphatic acyl radical of between 12 and about 30 carbon atoms and a composition comprising such a wax-like compound and a wax melting above about 100° F., said wax in such compositions not being present in an amount exceeding about four times the weight of said wax-like compound; (3) between about 0.5 and about 20 parts of a hydrophilic protective colloid free from rewetting tendencies after drying and (4) between about 0.5 and about 15 parts of an emulsifying agent of the group consisting of sulfonated and sulfated acids, alcohols and esters containing an aliphatic chain of between 8 and about 30 carbon atoms, sulfonated lignin, condensation products of polyalkylene polyamines with fatty acids containing between 8 and about 30

## 12

carbon atoms, dialkyl alkylol alkylamide quaternary ammonium salts and water-dispersible reaction products of an aliphatic amine containing from 8 to about 22 carbon atoms with epichlorohydrin.

6. A composition according to claim 1 containing from between about 1 and about 6 parts of an aliphatic alcohol having between 12 and 30 carbon atoms.

7. A composition according to claim 1 in which said resinous component is a methylated methylol melamine.

8. A composition of matter which comprises a stable aqueous dispersion of (1) between about 30 and about 600 parts by weight of methylated methylol melamine selected from the group consisting of water-soluble methylated methylol melamine and colloidal methylated methylol melamine; (2) 100 parts of a wax-like substance comprising paraffin wax melting above 100° F. and hydrogenated castor oil melting above 100° F. in a weight ratio not exceeding 4:1, paraffin wax to hydrogenated castor oil respectively; (3) between about 0.5 and about 20 parts of a hydrophilic protective colloid free from rewetting tendencies after drying; (4) between about 1 and about 6 parts of an aliphatic alcohol containing between 12 and 30 carbon atoms and (5) between about 1 and about 4 parts of a sulfated fatty alcohol containing between about 8 and about 30 carbon atoms.

9. A composition of matter which comprises an aqueous dispersion of (1) between about 30 and about 600 parts of a methylated methylol melamine selected from the group consisting of water-soluble methylated methylol melamines and colloidal methylated methylol melamine; (2) 100 parts of hydrogenated castor oil melting above 100° F.; (3) between about 0.5 and about 20 parts of polyvinyl alcohol and (4) between about 0.5 and about 15 parts of a sulfated fatty alcohol containing between 8 and about 30 carbon atoms.

10. A composition of matter which comprises a stable aqueous dispersion of (1) between about 30 and about 600 parts by weight of a mixture comprising a minor portion of a substance selected from the group consisting of water-soluble methylated methylol urea, methylol alkylene ureas and methylated methylol alkylene ureas, together with a major portion amounting to at least 30 parts of a methylated methylol melamine selected from the group consisting of water-soluble methylated methylol melamine and colloidal methylated methylol melamine; (2) 100 parts of a waxy substance comprising paraffin wax having a melting point above 100° F. and hydrogenated castor oil having a melting point above 100° F. in a weight ratio not exceeding about 4:1 paraffin wax to hydrogenated castor oil respectively; (3) between about 0.5 and about 20 parts of an hydrophilic protective colloid free from rewetting tendencies after drying; (4) between about 1 and about 6 parts of an aliphatic alcohol containing between 12 and about 30 carbon atoms; (5) and between 1 and about 4 parts of a sulfated fatty alcohol containing between about 8 and about 30 carbon atoms.

11. A process which comprises treating textile material with a composition according to claim 1 and a curing catalyst and heating the treated material whereby a durable water-repellent finish is imparted to the textile material.

12. A process which comprises treating a textile material according to claim 6 and a curing catalyst and heating the treated material whereby a durable water-repellent finish is imparted to the textile material.

13. An article which comprises a textile material having as a durable water-repellent finish the heat cured reaction product of a composition according to claim 1.

14. An article which comprises a textile material having as a durable water-repellent finish the heat cured reaction product of a composition according to claim 6.

## References Cited in the file of this patent

## UNITED STATES PATENTS

2,191,362 Widmer et al. ----- Feb. 20, 1940  
 2,197,357 Widmer et al. ----- Apr. 16, 1940  
 2,357,273 Thurston ----- Aug. 29, 1944  
 2,426,770 Grim ----- Sept. 2, 1947  
 2,536,978 Fordemwalt ----- Jan. 2, 1951

2,537,667 Harris ----- Jan. 9, 1951  
 2,835,639 Widmer et al. ----- May 20, 1958

## OTHER REFERENCES

5 Bennett: Commercial Waxes, pp. 91, 113, Chem. Pub. Co., Brooklyn, N.Y. (1944).  
 Swern et al.: J. Am. Chem. Soc. 67, 902-3 (1945).  
 Speel: Textile Chemicals and Auxiliaries, pp. 206, 207, 213, 299-316, 366-9 (1952).

UNITED STATES PATENT OFFICE  
CERTIFICATION OF CORRECTION

Patent No. 2,971,930

February 14, 1961

Nathaniel J. Glade

It is hereby certified that error appears in the above numbered patent requiring correction and that the said Letters Patent should read as corrected below.

Column 6, Table I, first column thereof, line 1, for "Slack was" read -- Slack wax --; columns 7 and 8, Table III, last column thereof, opposite Example 12, for "70" read -- 0 --.

Signed and sealed this 1st day of August 1961.

(SEAL)

Attest:

ERNEST W. SWIDER

Attesting Officer

DAVID L. LADD  
Commissioner of Patents